

July 16, 1946.

J. E. HENDERSON ET AL

2,404,343

PHOTOTUBES AND METHOD OF MANUFACTURE

Filed Oct. 14, 1943



*Fig. 1.*



*Fig. 2.*



*Fig. 4.*



*Fig. 3.*

INVENTORS  
JOSEPH E. HENDERSON  
BY & ROBERT B. JAMES  
Charles M. Clair  
ATTORNEY

## UNITED STATES PATENT OFFICE

2,404,343

PHOTOTUBE AND METHOD OF  
MANUFACTURE

Joseph E. Henderson, Seattle, Wash., and Robert B. Janes, Verona, N. J.; said Henderson assignor to the United States of America, as represented by the Secretary of Navy and said Janes assignor to Radio Corporation of America, a corporation of Delaware

Application October 14, 1943, Serial No. 506,274

10 Claims. (Cl. 250—165)

1

Our invention relates to photo-electric tubes and their method of manufacture, and particularly to tubes incorporating dual cathodes having coatings of elements such as antimony, arsenic and bismuth sensitized with an alkali metal.

In co-applicant Janes' copending application, Serial No. 434,681 filed March 14, 1942, there was described a phototube of a very rugged type capable of withdrawing high values of acceleration both longitudinally of the tube and when the tube is subjected to an angular acceleration, or centripetal acceleration such as exists when a whirling motion about its longitudinal axis is given to the tube. In this prior tube it was substantially impossible to obtain a very close spacing between the anode and cathode while still retaining its rugged character and high sensitivity. For example, co-applicant Janes found that it was necessary to separate the anode and cathode by a distance of at least three-quarters of an inch. Certain applications require closer spacing than this and, furthermore, such applications require the use of a second cathode which preferably serves as an anode to the first cathode.

It is an object of our invention to provide a very rugged phototube of the dual cathode antimony, arsenic or bismuth coated type. It is another object to provide a dual cathode phototube of the alkali metal treated antimony, arsenic or bismuth type, wherein the cathodes may be placed very close together. It is a further object to provide a phototube of the dual cathode type which will withstand high forces of acceleration without distortion or mechanical failure of the parts or variation in the operating characteristics of the tube while providing a structure which may be easily processed and having high photo-sensitivity. It is a further object to provide an improved method of manufacturing a very rugged phototube of the dual cathode antimony, arsenic and bismuth coated types. It is a still further object to provide a method of manufacture allowing the production of dual antimony coated cathodes without deterioration of the antimony coating or coatings during processing.

The foregoing and other objects, features and advantages of our invention will be apparent when considered in view of the following description and the accompanying drawing wherein,

Figure 1 is a view in longitudinal section of a phototube made in accordance with our invention.

Figure 2 is a cross sectional view of the phototube shown in Figure 1 taken along the lines 2—2.

Figure 3 is a sectional view of a modified electrode for use in the tube of Figure 1, and

2

Figure 4 is a longitudinal sectional view of apparatus suitable for performing one of the principal operations involved in the manufacture of the phototube hereinafter described.

5 In the following description we will refer specifically to antimony as a cathode coating and it will be appreciated that arsenic and bismuth are the full equivalents of antimony and may be substituted in whole or in part for the antimony without departing from the scope of our invention.

10 In accordance with our invention we have found that a tube comprising a tubular section or sections of insulating material and closed at 15 opposite ends by metal closure caps may be assembled with an additional cathode intermediate the closure caps if certain precautions are taken in the order of assembly and in the application of the antimony coatings on the cathode foundations, such as on one of the closure caps and the intermediate cathode foundation. More particularly we have found that a tube of the type described in co-applicant Janes' above-mentioned application may be constructed with an additional 20 photo-cathode intermediate oppositely disposed envelope closure caps serving as anode and cathode respectively with the two cathodes exceedingly close together, provided the cathode foundations are provided with their antimony 25 coatings following the sealing of the foundations or foundation supports in the tubular envelope.

30 Referring to Figure 1 wherein we have shown a phototube having dual cathodes made in accordance with our invention, the tube comprises two end closure caps 1 and 2, each of which is sealed to predetermined lengths of glass tubing 3 and 3a. The minimum axial length of the tubing 3 is not critical and may be considerably less than one-half inch although the minimum length 35 of the tubing 3a must not be less than one-half inch and is preferably not less than three-quarters of an inch. Preferably one of the caps, such as the cap 1, is apertured as shown at 4 and is provided with a glass tubulation 5 sealed around 40 the aperture for evacuation and so that following evacuation the tubulation may be closed such as by a tipping-off operation. The opposite closure cap 2 is non-apertured and supports a source 6 of alkali metal such as a caesium compound reducible to caesium upon the application of heat 45 to the central outer area of the cap 2.

50 In addition and in accordance with our invention we provide intermediate the closure caps 1 and 2 a second cathode foundation 7 at a distance preferably closer to the closure cap 1 than the clo-

sure cap 2. The foundation 1 serves both as an anode for the first cathode and, when further processed, as a cathode with respect to the cap 2. Further, in accordance with our invention the closure cap 1 supports a closely adjacent coating of antimony or an equivalent element facing in the general direction of the cap 2 but shielded therefrom by the second cathode foundation 7. As shown in Figure 1, the reasons for which appear more fully hereinafter, the second cathode foundation 7 is supported at a relatively short distance from the end cap 1 and at a larger distance from the end cap 2 by supporting means such as a ring-shaped or annular support member 8. It has been found that the foundation 7 cannot be photo-electrically sensitized with an alkali metal treated antimony, arsenic or bismuth coating if the distance between the end cap 2 and the coating is less than a predetermined minimum, such as less than one-half inch although this distance is preferably not less than three-quarters of an inch. However, in accordance with our invention we are able to provide very close spacings less than the minimum distance of one-half inch by following our improved method of manufacture. Since the cathode foundation 7 serves as a cathode with respect to the cap 2 and as an anode with respect to the end cap 1, and the end cap 1 is made photo-sensitive, the relatively close spacing between the foundation 7 and end cap 1 provides characteristics which were unobtainable in tubes of the types described using antimony coatings. Consequently, in accordance with our invention we provide, following the assembly of the end cap 1 to the glass tubing 3 and of the support ring 8 to both the glass tubing sections 3 and 3a, a coating of antimony 9 on the inner surface of the end cap 1 as shown in Figure 1, or on a foundation 10 supported by the end cap 1 as shown in Figure 3. Only then is the foundation 7 supported within the tube on the support ring 8, such as by welding metal tabs 11 between the foundation 7 and the support ring 8 or other mechanical attachment. The foundation 7 is provided with a coating 12 of an element such as antimony either before or after its attachment to the support ring 8 by the metal tabs 11.

More particularly we have found that it is not only desirable but necessary to provide the antimony coatings 9 and 12 at a definite time during the sequential manufacturing steps to prevent injury to these coatings during subsequent steps of the manufacturing processes. For example, if the coatings 9 and 12 are subjected to relatively high temperatures, such as occur when the closure cap 1 is sealed to the glass tubing 3 or when the support ring 8 is sealed between the tubular glass portions 3 and 3a, permanent injury occurs to the coatings. The sealing operations must necessarily be performed in the presence of normal atmospheric conditions and our sequence of processing steps avoids or substantially eliminates material oxidation of the antimony coatings on the foundations. Furthermore, the closure cap 1 and the support ring 8 must be subjected to certain processing steps to provide good sealing properties at the time the seals are made between these members and the glass tubings 3 and 3a, such steps being incompatible with previously applied antimony coatings.

The closure caps 1 and 2, as well as the ring member 8, are preferably of material such as chrome-iron having a co-efficient of expansion substantially matched with that of the glass of

the tubing 3 and 3a. A chrome-iron which we have found satisfactory for such use with lime glass contains as the principal constituents—

|            | Percent |
|------------|---------|
| 5 Chromium | 26-30   |
| Nickel     | 0.5     |
| Manganese  | 0.5     |
| Silicon    | 0.5     |
| Iron       | Balance |

10 Following formation of a closure cap 1 to a satisfactory form, one cap for each tube is apertured as shown at 4 and where a foundation member other than the cap for the first cathode is desired, such as the disc 10 shown in Figure 3, the disc 10 is attached to the cap 1, such as by welding. The material of the disc 10 as well as of the foundation 7 is preferably of high chromium content alloy such as chrome-nickel, the content of chromium ranging from 5 to 30% by weight, the alloy being oxidized to a greenish color as disclosed in Janes' copending application, Serial No. 481,246 filed March 31, 1943. The tubulation 5 is then sealed around the aperture 4 and the cap 1 oxidized to provide a film of oxide which forms a good bond between the cap 1 and the glass tubing 3 during the next operation of sealing these two parts together. Such oxidation may occur simultaneously with the sealing of the tubulation 5 to the cap 1, although alternatively the formed caps may be oxidized in moist hydrogen as described by Hull, Burger and Navis in an article entitled, "Glass-to-metal seals," part 2, Journal of Applied Physics, volume 12, No. 9, September 1941, pages 698-707. Such firing produces a relatively thick coating of greenish colored chromic oxide integral with the surface of the cap 1 and the disc 10, if such disc is used as the cathode foundation. If the moist hydrogen oxidation step is used we prefer to bake the end caps for a sufficient length of time, such as in a non-oxidizing atmosphere at a temperature of 500° C. for about twelve hours to remove any occluded hydrogen. The seal between the end cap 1 and the glass tubing 3 may be made by rotating the parts in the presence of fires heating the rim of the cap and the lower end of the tubing 3. We use a similar sealing step to attach the support ring 8 to the upper end of the glass tubing 3 and to the lower end of the glass tubing 3a. All of these steps are performed in accordance with our invention before the application of the antimony coatings 9 and 12, the cap 1 and the foundation 7 only then being ready for the application of the antimony coatings 9 and 12 which are applied in separate steps.

Referring to Figure 4 and prior to attachment of the foundation 7 to the ring member 8, we insert the glass tubing 3 and 3a over a tubular or cylindrical open ended shield 15, the shield extending to within close proximity of the end cap 1 or the disc 10, if such disc is used, and on which the antimony is to be deposited. The shield 15 is preferably supported within a chamber or bell jar 16 capable of being evacuated. We also support opposite the cap 1 a source of antimony to be vaporized and condensed thereon. Such a source of antimony may comprise a refractory metal coil 17 supporting a quantity of antimony 18 or other element such as arsenic or bismuth and which may be vaporized by passing an electric current through the connecting leads 19. Following the insertion of the open ended walls of the tube shown in Figure 1, the bell jar 16 is evacuated to a high vacuum, the residual air pressure preferably being less than 0.5 microns

and sufficient antimony is vaporized from the source 18 and condensed on the inner surface of the cap 1 to provide the antimony coating 9. The thickness of this antimony coating may range from a thickness corresponding to 0.1 to 0.16 milligram per square centimeter, which is sufficient to provide good sensitivity when such a coating is treated with alkali metal. The rate of vaporization and condensation is preferably low, being less than 0.2 milligram per square centimeter of the surface to be coated per second, since higher rates of condensation may be detrimental, forming a non-uniform coating. The entire bell jar assembly with the exception of the coil 17 and the heated antimony source 18 is preferably maintained at room temperature during the evaporation and condensation steps, except for such slight heating of the cap 1 as may occur by radiation from the coil 17.

The antimony coating 12 on the foundation 7 may be applied to a similar thickness in a similar manner either in the bell jar 16 following attachment of the foundation 7 to the ring member 8 by the metal strips 11, in which event the shield 15 is made somewhat shorter terminating adjacent the upper surface of the foundation 7, although the antimony coating 12 may be applied prior to its attachment while separately supported in vacuum with exposure to a heated antimony source. If this latter method is used the foundation 7 is affixed to the ring member 8 following the application of the antimony coating 12.

In accordance with our invention and following the application and assembly steps referred to above, the envelope formed by the tubular glass sections 3 and 3a is closed by sealing the cap 2 to the upper end of the tubing 3a at a sufficient distance, such as three-quarters of an inch from the surface of the nearest adjacent antimony coating, such as the coating 12. A source 6 of alkali metal such as a caesium bearing compound is first affixed to the inner surface of the end cap 2, such as by enclosing a compound of caesium in a small apertured container, whereupon the cap 2, previously oxidized as described above, is sealed to the upper end of the glass tubing 3a. To prevent excessive heating of the antimony coatings during this final sealing step, we prefer to cool the ring member 8 as well as the end cap 1, such as by a blast of air directed thereon during the sealing of the cap 2 to the upper end of the glass tubing.

The only other precaution which need be followed in the assembly of our dual cathode phototube is the maintenance of the antimony coatings in the absence of high concentration of water vapor, especially during the time these coatings are subjected to temperatures above normal room temperature. Consequently the relative humidity of the atmosphere to which the coated cathode foundations are subjected should be low and preferably less than 80% relative humidity at 25° C., which corresponds to a water vapor concentration equivalent to 8 grains of water vapor per cubic foot of air. The satisfactory results obtained are believed to be due to the fact that antimony does not oxidize when subjected to normal atmospheric conditions in the presence of low humidity.

Following the assembly of the tube as shown in Figure 1, the internal volume thereof is exhausted through the tubulation 5 and the tube is baked at a temperature of 275 to 310° C. to remove any occluded gases contained in the tube parts. Following this baking which may be from fifteen

minutes to one-half hour, we vaporize a quantity of alkali metal such as caesium from the source 6 to sensitize both of the coatings 9 and 12. To allow access of the alkali metal to the antimony coating 9 the foundation 7 is provided with an aperture 4a although sufficient spacing may be provided about the periphery of the foundation. Following the vaporization of the alkali metal the tube is baked, preferably at a temperature of 160° C., for thirty minutes and during this baking the alkali metal apparently combines with the antimony coatings to provide photocathode surfaces having very high sensitivity to light. Following the baking the tubulation 5 may be tipped-off and the tube removed from the pump and preferably rebaked at a temperature of 160° C. for a period of twenty minutes, following which the tube is aged to further stabilize the photoelectric emission from the cathode.

In operation the cap 1 serves as a cathode connection and is operated at a negative potential with respect to the ring member 8 which supports and is electrically connected to the cathode foundation 7, this member likewise being maintained at a negative potential with respect to the anode cap 2. The electrons liberated from the coating 9 are directly proportional to the light incident thereon through the glass tubing 3 and similarly electrons liberated from the coating 12 and collected by the anode cap 2 are directly proportional to the light incident on the coating 12 through the glass tubing 3a. Consequently the disclosed structure is ideally adapted to multi-directional use wherein either one or more light sources or a broad source such as the sky are used since the cathodes may be illuminated from all azimuths on sides facing the respective anodes.

While we have described our invention with particular reference to a dual cathode phototube and have set forth our preferred method of manufacturing such a tube, it will be appreciated that various modifications, such as multiple cathode phototubes, can be made both in the structure and in the method of manufacturing without departing from the spirit of our invention or the scope thereof as set forth in the appended claims.

We claim:

1. A phototube comprising a tubular glass envelope, a metal closure at each end of and forming the end walls of said envelope, a cathode foundation extending transversely of said envelope intermediate said closures, a coating selected from the group consisting of antimony, arsenic, and bismuth on the surface of said foundation facing one of said metal closures, a similar coating on the other of said closures and alkali metal within said envelope to sensitize said coatings.
2. A phototube comprising a tubular glass envelope, a metal cap sealed to each end of said envelope, a coating selected from the group consisting of antimony, arsenic, and bismuth on one of said metal caps as a cathode foundation, a second cathode foundation extending transversely of said envelope between said caps, a coating selected from the group consisting of antimony, arsenic, and bismuth on the surface of said foundation facing the other of said caps, and a quantity of caesium within said envelope to sensitize said coatings.
3. A phototube as claimed in claim 2 wherein said coatings are of antimony.
4. A phototube comprising a tubular envelope

of transparent material, a metal cap sealed to and closing each of the opposite ends of said envelope, a cathode foundation extending transversely of said envelope between said metal caps and being spaced more closely to one of said caps than the other cap, a coating selected from the group of elements consisting of antimony, arsenic and bismuth on said one of said caps and a second coating selected from said group of elements on the surface of said foundation facing the other of said caps, and an alkali metal deposited on each of said coatings to render said coatings photo-emissive.

5. A phototube comprising a cylindrical glass envelope, a metal cap at each end of said envelope, one of said caps being apertured and closed by an exhaust tubulation, a cathode foundation affixed directly to one of said caps and facing in the direction of the other of said caps, a second cathode foundation extending transversely across said envelope parallel to and between said caps and closer to said first cathode foundation than to the other end cap, and a coating of alkali metal treated antimony on each of said cathode foundations.

6. A phototube comprising a pair of coaxial, separated transparent envelope portions sealed at their adjacent ends to a metal support ring in a plane transverse to said envelope, a metal cap sealed to each of the opposite ends of said envelope portions, a coating of alkali metal treated antimony on one of said metal caps and a photo-sensitive electrode extending transversely across said envelope and supported by said metal support ring between said coating and the other of said metal caps and having a photo-sensitive surface facing said other metal caps.

7. A phototube comprising a pair of longitudinally spaced coaxial transparent envelope portions sealed at their adjacent ends to an electrode support member, one of said portions having an axial length less than three-quarters of an inch, the other having a minimum length of approximately one-half to three-quarters of an inch, a photocathode attached to and carried by said electrode support, a metal end cap closing the open end of each of said envelope portions and a coating of caesiated antimony on the cap sealed to that envelope portion whose minimum length is approximately one-half to three-quarters of an inch.

8. The method of manufacturing a phototube having two closure caps separated by a tubular insulating member and an intermediate electrode

comprising sealing one of said caps to one end of said member, sealing a support for a photo-sensitive electrode intermediate the ends of said member, depositing an element selected from the group consisting of antimony, arsenic and bismuth on a surface in electrical contact with the cap sealed to one end of said member, attaching an electrode foundation adapted to be photoelectrically sensitized to said support and then sealing the other cap to the other end of said member, evacuating the envelope formed by said member and said caps, and sensitizing said deposited element and said foundation with an alkali metal.

10. The method of manufacturing a phototube having an envelope of two metal closure caps sealed to and separated by sections of glass tubing comprising sealing one of said closure caps to one end of one of said sections of glass tubing, sealing a support for a photosensitive electrode to the opposite end of said one section, sealing one end of the other section of glass tubing to said support coaxial with said one section, depositing a coating of an element which when sensitized with an alkali metal is photo-sensitive on a surface adjacent said one closure cap, attaching a foundation which when sensitized with an alkali metal is photo-sensitive on said support, sealing the other closure cap to the other end of said other glass tubing section to form an envelope, evacuating said envelope and sensitizing said coating and said foundation with an alkali metal.

15. The method of manufacturing a phototube having two closure caps separated by tubular insulating material comprising sealing one of said closure caps to one end of said tubular insulating material, sealing an electrode support to said insulating material intermediate the opposite ends thereof, inserting an open-ended shield without in the open end of said tubular insulating material beyond said electrode support and to within close proximity of said sealed closure cap, evaporating and condensing antimony on a surface adjacent said closure cap while the inner walls of said insulating material and said electrode support are protected from condensation thereon by said open ended shield, removing said shield, attaching an antimony coated electrode to said electrode support, sealing the other closure cap to the open end of said tubular insulating material to form an envelope, evacuating said envelope and sensitizing said antimony with an alkali metal.

JOSEPH E. HENDERSON.  
ROBERT B. JANES.